

# UNITED STATES PATENT OFFICE.

BARNETT L. GEORGE, OF SALT LAKE CITY, UTAH.

## PROCESS OF CONCENTRATING ORES BY FLOTATION.

1,375,957.

Specification of Letters Patent. Patented Apr. 26, 1921.

No Drawing.

Application filed August 9, 1918. Serial No. 249,059.

To all whom it may concern:

Be it known that I, BARNETT L. GEORGE, a citizen of the United States, residing at Salt Lake City, in the county of Salt Lake and 5 State of Utah, have invented certain new and useful Improvements in Processes of Concentrating Ores by Flotation, of which the following is a specification.

This invention relates to improvements in

10 the concentration of mineral bearing ores, such as sulfid ores and the like, by means of the flotation process which is now carried out by subjecting the ore pulp to sub-aeration or to agitation in contact with air, after 15 adding to the pulp a quantity of oil or other suitable frothing agent, with or without the addition of an acid such as sulfuric acid, whereby a mineral bearing froth is formed which may be floated off. The present invention is based upon the discovery that the 20 flotation process is improved by the addition to the ore pulp of a quantity of zinc sulfate ( $ZnSO_4$ ). The improvement is particularly marked when the zinc sulfate is 25 used in conjunction with oils which give an organic acid reaction, although improved results are obtained when the reagent is used with oil giving an alkaline reaction.

The invention comprises the use of zinc 30 sulfate with various grades and kinds of oils, but the use of this reagent is especially advantageous in conjunction with light oils of crude coal tar, such as Barrett No. 4 creosote oil. This particular oil formerly 35 gave an alkaline reaction, and this alkalinity, though not enough to precipitate the tar acids, appeared to protect the oil from the acid in the pulp mixture, whereby the oil was capable of being more readily emulsified. The more recent output of Barrett 40 No. 4 oil gives an organic acid reaction and resists emulsification to a greater extent than the alkaline oil. The Barrett No. 4 oil of alkaline reaction gives excellent results in 45 conjunction with sulfuric acid, but the newer oil of acid reaction when used in the flotation process gives a tailing having a metallic content from 20% to 50% higher than that obtained when the corresponding 50 alkaline oil is used. When this Barrett No. 4 oil having an organic acid reaction is used without sulfuric acid, a tailing is obtained which is comparable with that obtained by the use of the alkaline oil, but it is found 55 that the froth builds up in the flotation ma-

chine and fails to discharge over the spitzkasten. The use of sulfuric acid provides the aeration necessary for the discharge of the froth, but if used with the oil having an acid reaction, it ruins the selective properties of the oil, and the selective properties of the oil of acid reaction when used with sulfuric acid have thus far not been improved by rendering alkaline the oil which gives the acid reaction.

60 However, I have found that zinc sulfate possesses the property of giving improved results when used either with an alkaline oil or an organic acid oil, such as the old Barrett No. 4 and the new Barrett No. 4 oil, for 65 example. Zinc sulfate is quite soluble in water and when introduced into the flotation machine as a solution it can be easily handled. It is comparatively cheap and compares favorably with sulfuric acid in cost 70 per ton of ore feed treated; it has the advantage over sulfuric acid that it gives an increase in the extraction of from 10% to 30%. Zinc sulfate possesses no selective 75 properties in itself, but it performs the function of sulfuric acid with improved results and with none of the injurious effects which the latter has upon the flotation machine.

80 In carrying out the process, the finely ground ore is mixed with water to form a 85 freely flowing pulp, and to this pulp there is added a small quantity of oil, such as Barrett No. 4 oil for example, together with a small quantity of zinc sulfate. The zinc sulfate is preferably added in the proportion 90 of from three to six pounds for each ton of dry ore feed treated, and the zinc sulfate solution may be added to the pulp mixture in the flotation machine. The mixture of pulp, oil, and zinc sulfate so formed 95 is then subjected to a flotation operation, in which the mixture is agitated and aerated to produce a froth which may be floated off from the spitzkasten or other separation vessel. A thorough emulsification of the 100 zinc sulfate, oil, and pulp, is necessary to procure the most satisfactory results. The quantity of zinc sulfate to be used for obtaining the best results will depend to some extent upon the method of carrying out the 105 flotation operation and upon the nature of the ore being treated.

110 The following example shows the comparative results following the use of Barrett No. 4 oil of the organic acid and the alka-

line type with sulfuric acid and with zinc sulfate in the concentration of a copper ore by means of the flotation process:

|                                                    | % Cu.<br>rougher<br>tails. |
|----------------------------------------------------|----------------------------|
| 5                                                  |                            |
| Alkaline Barrett No. 4 oil with sulfuric acid..... | .095                       |
| Alkaline Barrett No. 4 oil with zinc sulfate.....  | .105                       |
| Acid Barrett No. 4 oil and sulfuric acid.....      | .420                       |
| Acid Barrett No. 4 oil and zinc sulfate.....       | .120                       |

The foregoing example shows that zinc sulfate gives results with the acid oil nearly as good as those obtained with the alkaline oil, and both of these results are comparable to the results obtained with the alkaline oil and sulfuric acid, and very much better than the results obtained with organic acid oil and sulfuric acid.

It has been found further that when zinc sulfate is used as a reagent in the flotation process, the results are particularly improved when treating ores which do not readily yield to separation by flotation. The following is an example of the results obtained by the use of zinc sulfate as compared with sulfuric acid when treating a difficult copper ore feed:

|                                                                                 | % Cu.<br>rougher<br>tails. |
|---------------------------------------------------------------------------------|----------------------------|
| 30                                                                              |                            |
| Alkaline Barrett No. 4 oil and sulfuric acid.....                               | .430                       |
| Alkaline Barrett No. 4 oil and zinc sulfate.....                                | .180                       |
| Alkaline Barrett No. 4 oil and zinc sulfate with high sulfur<br>crude oil ..... | .145                       |

Zinc sulfate as a reagent in the flotation process appears to work substantially equally well with both the alkaline oil and the organic acid oil, and can be used beneficially with the organic acid oil, such as the new Barrett No. 4 oil, when sulfuric acid cannot. It gives a good extraction on an ore feed which is difficult to treat in cases where it has been found that the alkaline oil and sulfuric acid do not give a good extraction. It has further been found that when zinc sulfate is used with a mixture of crude mineral oil and coal tar oil, the froth is tender, well mineralized, and lively, where-

as, when sulfuric acid is used with these oils, there is a tendency to produce a similar condition of froth but the selective properties are comparatively poor.

Although I have described a particular method of carrying out my improved process and have given specific examples by way of illustration, it will be understood that the process may be altered in various ways without departing from the scope of the invention as defined by the appended claims.

What I claim is:

1. The process of concentrating ores, which comprises adding to an ore pulp an oil having an organic acid reaction and a quantity of zinc sulfate, and then subjecting the resulting mixture to a flotation operation.

2. The process of concentrating ores, which comprises adding to an ore pulp a quantity of light oil of crude coal tar having an acid reaction and a quantity of zinc sulfate, and then subjecting the resulting mixture to a flotation operation.

3. The process of concentrating ores comprising adding to an ore pulp from three to six pounds of light oil of crude coal tar having an acid reaction for each ton of dry ore feed, and then subjecting the resulting mixture to a floating operation.

4. The process of concentrating ores, which comprises mixing the finely ground ore with water to form a pulp, adding to the pulp a quantity of light coal tar oil having an acid reaction and a quantity of zinc sulfate, subjecting the mixture so formed to agitation and aeration, and separating the froth produced by the aeration of the mixture.

In testimony whereof, I have subscribed my name.

BARNETT L. GEORGE.